

## UNITED STATES PATENT OFFICE

ALBERT H. ACKERMAN, OF CHICAGO, ILLINOIS, ASSIGNOR TO CATALYTIC CHEMICAL COMPANY, OF DENVER, COLORADO, A CORPORATION OF COLORADO

## PROCESS OF TREATING FUEL OILS

No Drawing. Original application filed December 14, 1925, Serial No. 75,472. Divided and this application filed February 16, 1927, Serial No. 168,821. Renewed December 8, 1928.

This invention relates to a process for increasing the calorific value of fuel oils by causing the said oils to take up or dissolve certain quantities of petroleum coke.

- 5 Petroleum coke is a solid, black, more or less pitchy residue which is ordinarily produced in petroleum cracking stills and in similar operations where petroleum products are heated or distilled at a high temperature.
- 10 The petroleum coke remains after all the volatile materials have been driven off by the heating.

Now I have discovered that by the use of certain chemical reagents that will be described more fully below, I can cause this petroleum coke to dissolve or at least to disperse in fuel oil, so that the resultant mixture will be fluid and can be used in the same way as the untreated fuel oil, but the mixture

20 will have a higher calorific value due to the dispersed carbon therein contained.

The chemical reagents which I employ for this purpose are of such a nature that when used on mineral oil products which contain

25 viscous, waxy or pitch like and bituminous material, will cause such material to pass into solution in the oils.

In my patent, application Serial No. 75,472, filed December 14th, 1925, I have described a combination of materials which I employ for the treatment of heavy petroleum residues, for the treatment of cracking still residuum, for treating lubricating stock and in general for breaking up cluster of hydrocarbons contained in heavy mineral oils. This composition consists of mixtures of anthracene, sulfuric acid, oil of mirbane, sodium hydroxide, naphthalene in or about the following proportions:

|                         | Per cent |
|-------------------------|----------|
| 10 lbs. anthracene      | 4.61     |
| 4 lbs. oil of mirbane   | 0.92     |
| 2 lbs. sulfuric acid    | 1.82     |
| 1 lb. sodium hydroxide  | 0.45     |
| 45 200 lbs. naphthalene | 92.20    |

In case pure 85% anthracene is employed I can omit the sulfuric acid, which is used solely for the purpose of treating the anthracene when the 40% commercial grade of this

substance is employed, as it appears to increase the activity of the anthracene.

In making the aforesaid composition I proceed by first mixing the anthracene with the sulfuric acid allowing the action to proceed for a short time. The anthracene becomes much darker in color. If 85% anthracene is used, this treatment can be omitted. Thereupon, I add the oil of mirbane and then the sodium hydroxide, and grind the resultant pasty mixture. Most of the sulfuric acid will be neutralized by this treatment. The mixture is then allowed to stand for about one hour. This mixture is then added to the naphthalene and the whole material thoroughly ground, preferably in a ball mill, until the mass is uniform. The mixture is then packed in airtight containers for shipment and use.

The petroleum coke is incorporated with fuel oil by the aid of my aforesaid composition. I have found that by grinding up petroleum coke and adding to it a reasonable amount (say from 10-15% by weight) of my composition of materials and grind further, that the resultant mixture of coke and chemicals will dissolve to quite a considerable extent in common fuel oil and that the coke will likewise be dissolved so that the thermal efficiency of the fuel oil will be increased by from thirty to thirty-five percent in heat energy as measured in calories or British thermal units. I am not aware that such treatment of petroleum coke has ever been considered before.

The fuel oil may be of the kinds commonly used, and the incorporation of the coke, chemicals and oil may be carried out in any suitable type of mixing tank, preferably one having some means for agitating the contents of the tank.

What I claim is:

1. The process of treating fuel oil to increase the efficiency thereof which comprises comminuting petroleum coke with a composition of materials comprising naphthalene, anthracene, oil of mirbane, sulfuric acid and sodium hydroxide, and adding the same to the fuel oil and agitating the fuel oil.

2. The process of treating fuel oil which

comprising grinding petroleum coke with a composition of materials comprising naphthalene, anthracene and oil of mirbane, and thence adding the co-mixed coke and composition of materials to the fuel oil.

3. A process for incorporating petroleum coke with fuel oil comprising grinding said coke with a mixture of anthracene, naphthalene, oil of mirbane and sodium hydroxide, adding the resultant mixture to fuel oil and agitating the fuel oil to cause the admixed material to dissolve.
4. The process for incorporating petroleum coke with fuel oil which comprises grinding a major portion of petroleum coke with a minor portion of a composition of materials comprising substantially 10 parts anthracene, 4 parts oil of mirbane, 2 parts sulfuric acid, 1 part sodium hydroxide and 200 parts naphthalene, adding the resultant mixture to fuel oil, and agitating the fuel oil to cause the admixed material to dissolve therein.

5. The process for incorporating petroleum coke with fuel oil which comprises grinding a major portion of petroleum coke with a minor portion of a composition of materials constituting the reaction product resulting from the admixture of substantially 10 parts of anthracene, 4 parts oil of mirbane, 2 parts sulfuric acid, 1 part sodium hydroxide and 200 parts naphthalene, adding the resultant mixture to the fuel oil and agitating the same to cause the admixed material to dissolve therein.

In witness whereof, I have hereunto subscribed my name.

ALBERT H. ACKERMAN.

40

45

50

60

65